

E. P. GUINAT.  
SOLIDIFYING PROCESS FOR INGOTS.  
APPLICATION FILED JULY 3, 1903.

909,556.

Patented Jan. 12, 1909.

3 SHEETS—SHEET 1.

Fig. 1.



Fig. 3.



Fig. 4.



Fig. 2.



Fig. 4.



Fig. 5.



Fig. 6.



Fig. 8.



Fig. 7.



Fig. 9.



WITNESSES :

W. M. Avery  
P. J. Caramagh.

INVENTOR  
Eugène Paul Guinat  
BY

ATTORNEYS.

E. P. CUINAT.  
SOLIDIFYING PROCESS FOR INGOTS.  
APPLICATION FILED JULY 3, 1903.

909,556.

Patented Jan. 12, 1909.

3 SHEETS—SHEET 2.

*Fig. 10.*



*Fig. 11.*



WITNESSES

W. M. Avery  
R. B. Donaghay.

INVENTOR  
Eugène Paul Cuinat  
BY

ATTORNEYS.

E. P. CUINAT.  
SOLIDIFYING PROCESS FOR INGOTS.  
APPLICATION FILED JULY 3, 1903.

909,556.

Patented Jan. 12, 1909.

3 SHEETS—SHEET 3.

Fig. 12.



Fig. 13.



WITNESSES :

W. M. Avery  
R. D. Caramagh.

INVENTOR  
Eugène Paul Cuinat  
BY

Wm. C. C.

ATTORNEYS.

# UNITED STATES PATENT OFFICE.

EUGENE PAUL CUINAT, OF UNIEUX, FRANCE.

## SOLIDIFYING PROCESS FOR INGOTS.

No. 909,556.

Specification of Letters Patent. Patented Jan. 12, 1909.

Application filed July 3, 1903. Serial No. 164,187.

To all whom it may concern:

Be it known that I, EUGENE PAUL CUINAT, of the Steel Works, Unieux, Loire, Republic of France, engineer, have invented a Solidifying Process for Ingots, of which the following is a full, clear, and exact description.

The present invention relates to a process of compressing, forging and rolling steel ingots after their withdrawal from the molds but before they have completely hardened or solidified.

All processes hitherto invented for compressing ingots which have not hardened or become solid consist in effecting this compression in the mold into which the metal has just been poured. This process might be satisfactory if it was not only a matter of suppressing the hollow due to shrinkage but also to prevent flaws or air holes, but as at present by a judicious addition of silicon, manganese and above all by the employment of aluminum it is possible to obtain steel free from flaws or air holes and the problem to be solved is confined to preventing shrinkage taking place during solidification of the metal and thus to realize a considerable economy in the loss of height which this shrinkage necessitates at the upper part of the ingots. Now this result may be obtained by processes which are more simple, more rapid and less costly than those hitherto in use by operating direct upon the ingot which has been withdrawn from its mold instead of compressing it in its mold.

The principle of this new process is as follows:—It is known that in its transition from the molten to the solid state, steel passes through an intermediate state in which it consists of grains already solidified surrounded by a cement still fluid and has only the consistence of fresh mortar made from sand and quick lime, so that it opens and disintegrates under the influence of the slightest effect of extension.

Figure 1 is a section of an ingot immediately after it is cast and in the earliest stage of the process; Fig. 2 is also a section of an ingot, but representing the solidifying process as somewhat more advanced; Fig. 3 represents a more advanced stage of the process, the ingot being represented in section, as before; Fig. 4 is a view similar to Fig. 3, but representing the process as still further advanced; Fig. 5 is a diagrammatic view, representing the ingot as about to be pressed

on all sides; Fig. 6 is a plan of an ingot, showing the form which it would take when the resulting ingot was to be substantially square in section with flat faces; Fig. 7 is a plan of an ingot having convex faces when cast, the resulting ingot having flat faces; Fig. 8 is a plan representing a finished ingot with concave faces, the same having flat faces when originally cast; Fig. 9 represents an ingot of the general form in Fig. 7, this ingot having, however, concave faces formed from flat faces by a pressure. Fig. 10 represents partly in section and partly in elevation, a press to compress the ingots in the manner above described; Fig. 11 is a plan of the same apparatus; Fig. 12 is a view partly in section and partly in elevation of a modified form of press in which the pressure is applied by means of rollers or cams; Fig. 13 is a plan of this modified construction; Fig. 14 is an elevation partly in section; and Fig. 15 is a plan of another modification.

In these figures the same letters designate the same parts.

In order that the invention may be more clearly understood I have shown at Fig. 1 the section of an ingot just cast; in this figure the part which is cross hatched with oblique lines indicates the metal which has already solidified; the part indicated by slots represents that portion of the metal where the structure consists of grains. The horizontal lines represent the steel which is still liquid or molten. It is seen that at this time the portion of the ingot which has completely solidified is so thin in places that it would break under a very small strain; it thus results that it would not be considered possible to take the ingot out of the mold and to manipulate it in this state. But if a few minutes are allowed to pass (the number of which vary with the size and form of the ingots) the conditions are changed as shown in Fig. 2. The exterior is then completely solidified and has become much thicker; in the granular portion above referred to, the cement has congealed around the grains; by this fact that portion hatched with oblique lines is transformed into steel which is forgeable, tenacious, plastic and capable of supporting, without breaking or cracking, elongations and deformations much more considerable than the same metal would support in a cold state; at the same time

the ingot has also acquired a certain tensile resistance.

The metal as much granular as molten in the interior of the ingot is surrounded with an envelop still plastic, somewhat solid and somewhat tenacious which retains it. This enables the ingot to be withdrawn from its mold without inconvenience and to be carried in a vertical position to an apparatus 10 arranged for the purpose where it is submitted to lateral pressure without fear of causing it to crack. If this pressure is applied commencing towards the base of the ingot, the steel which is granular or fluid is 15 caused to rise towards the top and to fill up the hollow which would be left there by shrinkage, during which the contact of the cold tools at the same time as local applications of water (either in the form of spray 20 or jets) or any other refrigerating means causing the oxid which is formed on the metal to be cleaned off, will hasten the solidification of the interior metal.

The operation may thus be accelerated at 25 will, which improves the metal by preventing crystallization and eliquation which result from a slow cooling, so that if the pressure is gradually increased towards the top there will be obtained, if the operation is

30 carefully performed a full strong ingot. Figs. 3 and 4 represent longitudinal vertical sections of an ingot after two applications of successive pressure and Fig. 5 a diagrammatic view of the pressing tools *d* arranged 35 around the ingot *a* upon which the deformations produced are indicated in dotted lines. These deformations having only to compensate for the volume of shrinkage in the interior will not be considerable so that it is 40 only necessary to compress the faces of the ingot without touching the angles as shown at Fig. 5. The cast ingots may have given to them a form which will facilitate their compression. It will generally be an advantage 45 to make the sides of the ingot mold slightly concave so as to obtain ingots slightly convex as shown in Fig. 6 for ingots to have a square section and as shown at Fig. 7 for flat ingots. This convexity will 50 be calculated in such a way that by reducing the surfaces to a flat state, it will compensate for the interior shrinkage.

Flat ingots for making into sheets will 55 only need to be compressed upon their two large surfaces, the cooling of the small sides being effected by sprinkling of water. However if there is no objection to having ingots the sides of which are hollow after compression as shown in Figs. 8 and 9, there is no 60 reason why they should not be cast with flat or slightly concave faces so that these latter may be caused to enter more easily by the compression, the metal will stand the necessary extension without cracking.

65 For all ingots of small dimensions, it will

be more simple to take the ingot out of its mold and to transport it in a vertical position to the compressing apparatus. Ingots a larger size should on the contrary be cast upon a movable carriage which will permit 70 it to be transported with its mold under the apparatus which will remove the mold and afterwards under the compressing apparatus which will only be movable in a vertical direction. The compression may be effected 75 in different ways and the arrangements may be varied according to the form and weight of the ingots.

The accompanying drawings show by way of example three modified forms of apparatus 80 capable of realizing this method of compression.

The method of compression above referred to may be carried into effect by several arrangements the principal of which 85 are: 1. A system of presses acting on each side of the ingot which remains a fixture. 2. A system of small rollers or cams between which the ingot is pushed which causes the rollers or cams to rotate. 3. A 90 rolling mill for use with flat ingots having two cylinders between which the ingot is caused to travel by the rotary movement of the two cylinders.

The system of hydraulic or other presses 95 is shown in Figs. 10 and 11. It consists of four presses arranged at right angles to each other. Each consists of a cylinder *b* and a piston *c*. The four cylinders are in communication with each other so that when 100 one receives the water under pressure the others receive it at the same time. Each piston is provided on one face with pump leather and on the other with a forging tool *d*. It is guided above and below by rods *e* 105 in the form of bolts which connect it to a spring *f* which has a constant tendency to cause the piston to enter the cylinder. The ingot *a* is shown on its base in the center of this system of presses. The chains or 110 links *g* connect this apparatus with a crane which permits it to be moved vertically so as to vary the point at which the pressure is applied to the ingot, as above described. A current of water for cooling is shown at *h* 115 acting in conjunction with the presses.

The operation is carried out in the following manner. When the ingot has been cast a certain time is allowed to pass, variable according to its weight, it is then taken out 120 of the mold and conveyed under the press, a series of progressive compressions is applied between which compressions successive vertical displacements of the apparatus take place traveling in an upward direction; little 125 by little the lateral sides of the ingot are compressed thus preventing the formation of any hollows due to shrinkage.

The system by means of compressing rollers or cams is shown in Figs. 12 and 13. It 130

consists of four rollers or cams *i* facing each other and arranged at right angles, each of which is movable on its axis. They are each provided at *j* with a recess to permit the ingot to be readily engaged. The center of the apparatus is placed below the hydraulic or other press *k*. Before the machine is put into operation, the cams or rollers are arranged so that the recesses *j* are all facing 10 one another as shown in the drawing; the ingot taken from its mold and still molten in its interior is placed in position and it is caused to descend by means of the ram *k* until it passes out of the bottom of the apparatus. The ingot causes the cams or rollers to rotate and is thus compressed laterally from below upwards during which the cooling current *h*, hastening the cooling of the ingot, permits the compression to be accelerated. 20

The apparatus having only two rollers or cams is shown diagrammatically at Figs. 14 and 15. These two rollers *l* are analogous to those employed in rolling mills; they have 25 each a depression *m* enabling the ingot to be readily engaged. The two rollers acted upon simultaneously by any suitable gearing are placed so that the depressions are face to face. The ingot *a* is placed in position and 30 it is drawn downward by the rotation of the rollers and compressed upon its two large faces. A current of water *h* accelerates the cooling and prevents the sides which are not

sustained bursting under the action of the internal pressure.

35

Special attention is called to the fact that the effect of the cooling water is local, operating to form a thin shell around the inner plastic or molten ingot. If this shell were not formed, the pressure on the sides 40 of the ingot would have only a surface effect. However, on account of the presence of this shell, the pressure on the sides of the ingot does not affect the surface locally so as to disturb its structure, but simply forces the 45 shell inwardly as though it were a compressing plate. In this way the molten interior of the ingot is forced upwardly and piping is prevented.

50

Claim.

The process of solidifying ingots having a fluid interior which consists in spraying the side walls thereof to produce a sudden cooling, and to form a hard external shell, and simultaneously pressing said shell 55 inwardly upon the soft interior to weld together the inner parts of the opposing side walls at a high temperature.

The foregoing specification of my "Solidifying process for ingots" signed by me 60 this sixteenth day of June, 1903.

EUGENE PAUL CUINAT. [L. S.]

Witnesses:

J. ALLISON BOWEN,  
RENÉ CHIRIOT.